

# UNITED STATES PATENT OFFICE.

JOSEPH J. SACHS, OF MANCHESTER, COUNTY OF LANCASTER, ENGLAND.

## PREPARING AND BLEACHING JUTE.

SPECIFICATION forming part of Letters Patent No. 244,674, dated July 19, 1881.

Application filed July 1, 1880. (No model.) Patented in England June 16, 1880.

*To all whom it may concern:*

Be it known that I, JOSEPH JULIUS SACHS, of Manchester, in the county of Lancaster, England, have invented certain new and useful Improvements in Decoloring Jute, China Grass, and other Vegetable Fibers, of which the following is a specification.

My said invention relates to the treatment of vegetable fibers—such, for example, as jute, China grass, hemp, flax, and other like fibers—in order to render them curly and elastic, more pliable and less colored, and therefore more suitable for spinning, weaving, dyeing, manufacturing paper, felt, and for other purposes, either alone or mixed with other fibers of vegetable or animal origin.

According to my said invention I cut the fibers in lengths varying, according to the purpose for which they are to be used, from, say, one and one-half inch to two or three inches in one case, and from about six to twelve or eighteen inches in other cases. After or previously to this operation I separate the adhering fibers by pressure applied by elastic or other rollers, or by any other suitable means. The fibers thus prepared are then treated with a bleaching agent in solution—such, for example, as bleaching-powder, chlorozone, or similarly-acting agents, or potassium, permanganate, the latter being followed by a suitable acid—such, for example as hydrochloric acid, oxalic acid, sulphurous acid, and the like. After the bleaching solution has been drained off or otherwise removed the fiber is brought into a curly and more elastic state by introducing into it a solution of caustic soda or potash, or of any other material which will cause the fiber to contract and to curl—such, for example, as zinc chloride, dilute sulphuric acid, and the like. In order to modify the contracting and curling action of these substances, I sometimes add to the caustic solution small quantities of other substances—such, for example, as borax, sodium silicate, ammonia, and the like—in the proportion of, say, from about one-quarter to one-half per cent. of the weight of the solution, according to the qualities of the fibers and the kind of modification intended. The solutions should be of sufficient strength to act upon the fiber in the manner hereinbefore described. For example, the solution of caustic

soda should contain, say, from about ten to thirty per cent. of sodium hydrate, (NaOH,) according to the quality of the fibers. The fibers remain in the solution until they appear to be sufficiently curly, which result will usually be accomplished in, say, from about two to ten minutes. The fibers are then freed from the solution by any suitable means—as, for example, by squeezing between rollers, or by the use of an hydro-extractor or otherwise—and are next treated with suitable neutralizing agents—as, for example, in case of caustic alkalies having been used, with acids, such as muriatic or sulphuric acid or the like, and in case of acids having been used in order to contract and cure the fibers, with alkalies, alkaline salts, ammonia, and the like—which neutralizing agents are afterward removed by washing, the fiber being subsequently dried either at the usual or at an elevated temperature.

The fibers treated in the manner hereinbefore described offer great facilities for dyeing and printing, either used alone or mixed with other fibers, especially with those of animal origin, which qualities, combined with their curly wool-like appearance, render them very valuable in the production of imitations of textile fabrics, especially as they can be combed and spun together with other (and particularly animal) fibers—such, for example, as wool and the like.

Having now described my said invention and the manner in which the same is or may be used or carried into effect, I would observe, in conclusion, that I am aware that it has previously been proposed to treat fibers with a solution of caustic soda; but in such cases the fiber has been operated upon in its natural length, and has been submitted to the action of the solution for a protracted period, and has, moreover, been subjected to a multiplicity of preliminary and subsequent processes involving great expense. I lay no claim, therefore, to the use of a solution of caustic soda, except when the fibers are prepared for such solution and operated upon therewith, as herein set forth; but

What I consider to be novel and original, and therefore claim herein, is—

The method of rendering vegetable fibers curly, more pliable, and less colored, and therefore more suitable for spinning, weaving, dye-

ing, and printing, by subjecting them, after cutting into lengths and bleaching, to the action of caustic soda or potash or other liquid of the character and strength described, and then neutralizing and expressing the liquid, substantially as set forth.

In testimony whereof I have signed my name

to this specification in the presence of two subscribing witnesses.

J. JULIUS SACHS.

Witnesses:

FREDK. C. DYER,  
CHAS. MILLS,

*Both of 47 Lincoln's Inn Fields, London.*